

# UNITED STATES PATENT OFFICE

ALBERT J. RYAN, OF CINCINNATI, OHIO, ASSIGNOR TO RYAN IDEAL STAIN AND BLACKING COMPANY, OF LYNN, MASSACHUSETTS, (A FIRM COMPOSED OF ALBERT J. RYAN, OF CINCINNATI, OHIO, AND ALEXANDER J. McCORMICK AND DENNIS F. MARKS, BOTH OF LYNN, MASSACHUSETTS.)

## BOX MATERIAL FOR BOX-TOES OR THE LIKE FOR SHOES.

1,269,647.

Specification of Letters Patent. Patented June 18, 1918.

No Drawing.

Application filed September 8, 1914. Serial No. 860,550.

To all whom it may concern:

Be it known that I, ALBERT J. RYAN, a citizen of the United States, and a resident of the city of Cincinnati, in the county of Hamilton and State of Ohio, have invented certain new and useful Improvements in Box Material for Box-Toes or the like for Shoes, of which the following is a specification.

10 In the manufacture of shoes in the past, it has been the practice to supply for the stiffened portion of the shoe such as the box toe, a piece of material known as box material, which has been treated with certain 15 gums and waxes which will harden when dry. Accordingly in making up the shoe, this gum is placed on the box portions and the shoe lasted and set aside to dry for several days. A composition of waxes has also 20 been discovered which may be put on the box portions to harden them, and then these portions softened up before use, by high temperatures. Several days are required to 25 harden these articles also, but the danger of getting gum and wax on the shoe is done away with. Then, for a further step, a composition has been put on the market with 30 which to harden box toes or the like, which will become soft when treated with live steam, and will be rehardened almost immediately.

Now in the lasting of a shoe, it is necessary after the preliminary pulling over of the parts on the last, to wipe in the shoe by 35 inserting it with the last in a machine for that purpose. If the toe portion is wet and gummy, this wiping in will injure the shoe because of exuding matter. If the box portions are of the quick hardening material, 40 they will be too hard after the pulling over to go to the wiper.

In the latter kind, therefore, the shoe must be subjected to a second treatment of steam before wiping in is done, and with any 45 chance extra pressure or slight carelessness the steam may become so hot as to permanently injure the leather of the shoe, although at dry heat shoe leather will crack lower than with live steam heat.

50 It is the object, therefore, of my invention to furnish a box material for box toes or the like, which will soften at a moderate temperature of say one hundred and seventy-five

to two hundred and twenty-five degrees Fahrenheit of dry heat, and will quickly ~~as~~ harden upon cooling. No shoe leather will reach the point where it will crack at dry heat of two hundred and twenty-five degrees Fahrenheit.

Such a composition material is valuable ~~or~~ for making models of shoes from patterns also, constructing the whole shoe or the principal parts thereof of this material, such material adapted to be handled by the operator in the presence of a non-injurious heat ~~or~~ and hardened piece by piece at will.

I have discovered that a gum commonly known as "bold black gum" is perfectly adapted for the purpose intended, and in order to provide my new box material I take 70 sheets of felt, canvas, leather or other permeable material, and thoroughly saturate the same with bold black gum dissolved in a suitable solvent such as benzol or naphtha. The web, preferably of felt, is treated with 75 the gum solution in any convenient way until it is thoroughly saturated with the bold black gum, which at once hardens, leaving the sheet in a hard, firm, flexible condition from which the shoe forms, box toes and 80 such can be readily and easily cut of the proper size and shape for use, or the box material can be sold commercially in flat sheets to shoe manufacturers.

"Bold black gum" is a mineral product, so far as I am informed, similar to asphaltum for example, which is imported to this country from Australia under the above name. It comes in chunks the size of an egg. It has a high melting point in its natural state, 90 such as to make it impossible to dip felt into it, but when treated with naphtha or benzol seems to change its nature so as to have the melting points hereinafter noted.

The important feature of the invention 95 and the novel element is not the fact that a hardened blank is made, which is old, but that the hardened blank has the characteristics of softening at a fairly low temperature and immediately hardening when 100 allowed to cool. The box material softens so that it can be properly worked at a temperature from one hundred and seventy-five to two hundred and twenty-five degrees Fahrenheit without running or becoming 105 gummy or sticky, and as soon as the heat is

removed, it hardens in a few minutes or less to its normal stiff and flexible condition.

The temperature of one hundred and seventy-five to two hundred and twenty-five degrees Fahrenheit is not so high that the wearer of the shoe will encounter any such temperatures, and if he does, the shoe will retain its shape if nothing else occurs but the heating.

Having thus described my invention, what I claim as new and desire to secure by Letters Patent, is:

1. A box material for box toes or the like for shoes comprising a piece of material permeable to gums and waxes in general, said material permeated with a solution of bold black gum and a suitable solvent.

2. A box material for box toes and the like for shoes comprising a piece of material permeable to gums and waxes in general, said

material permeated with a composition comprising a gum hard at normal temperature, and a solvent of benzol or naptha, which composition softens at from 175° to 225° F. without running, and hardens at once at normal atmospheric temperatures.

8. A box material for box toes and the like for shoes comprising a piece of material permeable to gums and waxes in general, said material permeated with a composition comprising a gum hard at normal temperature, and a solvent of benzol or naptha, which composition softens at from 175° to 225° F. without running or becoming sticky, and hardens at once at normal atmospheric temperatures.

ALBERT J. RYAN.

Witnesses:

FRANK W. KUNKEL,  
KATHERINE SMITH.